

# UNITED STATES PATENT OFFICE.

WERNER SPALTEHOLZ, OF LEIPZIG, AND KURT HARING, OF HERSFELD, GERMANY,  
ASSIGNORS, BY MESNE ASSIGNMENTS, TO THE CORPORATION ANLYDAT-LEDER-  
WERKE, AKTIENGESELLSCHAFT, OF HERSFELD, GERMANY.

## MANUFACTURE OF LEATHER AND PRODUCTS RESEMBLING LEATHER.

1,200,146.

Specification of Letters Patent.

Patented Oct. 3, 1916.

No Drawing.

Application filed December 13, 1912. Serial No. 736,533.

*To all whom it may concern:*

Be it known that we, WERNER SPALTEHOLZ, and KURT HARING, both citizens of the German Empire, and residents of Leipzig (with the post-office address Mozartstrasse 21) and Hersfeld, Hesse-Nassau, (with the post-office address Doppelstrasse 4,) Germany, respectively, have invented new and useful Improvements in the Manufacture of Leather and Products Resembling Leather, of which the following is a specification.

The present invention relates to the manufacture of leather and leather-like products and has for its object the production of leathers having improved qualities such as to make them of increased value for ordinary uses and to render them useful for purposes for which ordinary leathers are not adapted.

The invention may be considered as a development and enlargement of the invention set forth in our United States Letters Patent No. 1,066,231, July 1, 1913, and consists generally speaking, in dehydrating a hide or skin or a preliminarily tanned leather and subsequently tanning the dehydrated material by a suitable molten agent in such a manner that the pores of the material become substantially completely filled with the agent. The agent should be one which becomes liquid at temperatures not injurious to the hide fiber but considerably above the temperature at which the leather is to be used.

The dehydrating is preferably accomplished by immersion in baths of alcohol, acetone or the like of successively increasing strengths, and the treatment with the molten tanning agent is preferably preceded by a treatment with a non-aqueous solution of resinous material. In the latter case a diffusion of the solution in the pores and the molten material takes place, the solvent being removed meanwhile as by evaporation, and the resulting product is to a high degree non-porous.

Our invention has especial application to the improvement of chrome leather. For example, if the leather tanned in the usual manner and not yet stuffed with fat is treated with an agent adapted to take the place

of water, such as alcohol, a new and valuable product is obtained, which has the particular characteristic that it need not be fat- 55 ted in order to prevent its drying hard. Moreover, this product is considerably im- 60 proved if it is treated with a solution, say, in alcohol, of a suitable material which is insoluble in water, or with such material in molten condition or with such solution fol- 65 lowed by treatment with such molten mate- rial.

A specific example of our process as applied to chrome leather is now given, it being understood, of course, that various modifications may be made by one skilled in the art without departing from the spirit of the invention.

Example 1: The hides unhaired in the usual manner by means of lime water are chrome tanned by the one bath process or by the two bath process. After the hides are tanned through, they are not, as is usual stuffed with fat before drying, but are 75 stretched on frames and placed in a bath of alcohol of about 60 per cent. strength and then transferred successively to two or three baths of stronger alcohol, the last being of 90-96 per cent. strength. The skins should 80 be left in each bath for 24 hours, but this time can be considerably shortened by agitating either the hides or the bath. After all the water has been exchanged for alcohol, the latter is distilled from the hides in a 85 vacuum of 100 to 50 mm.—about  $\frac{1}{2}$  to  $\frac{1}{15}$  atmospheric pressure—and at a temperature of 28-35° C. The product obtained is characterized by great pliability and is of additional and special value for all purposes in 90 which the presence of fat or oil or the like is not permissible, for example, for motor vehicle tires.

A further treatment of the above product may be carried out as follows, for the purpose of improving the quality thereof, especially to make it waterproof. The hides dried by vacuum distillation and containing practically no water are placed in a solution of resin or the like in a suitable solvent, such as alcohol, aceton, benzene, benzin or turpentine, carbon disulphid, carbon tetrachlorid, in a word, in any non-aqueous solvent. The dissolved substances which can be intro-

- duced into the hide in this manner are widely varied; for example shellac, colophony, mastic, in fact any resin that is soluble, also caoutchouc, guttapercha, cellulose derivatives, bituminous substances, residues from the dry distillation of coal tar and lignite tar, and even such tar itself dissolved in suitable solvents may be used, or mixtures of any of these materials in suitable proportions. All these substances have, so far as tanning is concerned, a common property which they retain in the leather treated with them, namely they are insoluble in water.
- 15 For the purpose principally of obtaining a softer leather than would be produced were resins, asphalts and the like used alone, it is advantageous to add to such materials, liquid or semi-liquid substances such as oils, 20 for instance, linseed oil, varnishes, for instance, linseed-oil varnish, vaseline and paraffin wax. Especially good results are obtained by using substances having an asphaltic base such as natural asphalt and artificial asphalt (petrol-goudron) dissolved 25 in benzene. By mixing artificial asphalt with natural asphalt or by mixing artificial asphalt having a high melting point with artificial asphalt having a lower melting 30 point or by the addition of one of the aforesaid liquid or semi-liquid softening substances to either kind of asphalt, a leather of any desired softness and pliability may be obtained.
- 35 When the products are made only with a solution as described, the evaporation of the solvent again produces small cavities in the product and the leather while waterproof to a considerable degree is not impervious to 40 water under pressure. If this is to be avoided, either a solvent is not used and the material is applied in the molten condition, or the process with the dissolved tanning material is used as a preliminary treatment, a 45 further tanning being afterward effected by means of a molten material, asphalt being in the fore-front in this respect.
- 50 A form of the process will now be described, in which first a solution of the tanning material is used and then a fused material.
- 55 Example II: The raw hide or chrome leather or fatted (or fatted and subsequently defatted) bark tanned leather at any stage of the tanning process, or iron tanned or alum tanned leather, dried with alcohol and dehydrated in a vacuum, is placed in a solution of a resin or a bituminous substance in a non-aqueous solvent, 60 preferably artificial asphalt in benzene and is left there until thoroughly soaked; this may take from 3 to 14 days according to the solution used. The concentration of the solution may be between 38 and 50 per cent. 65 according to the viscosity of the fluid formed.

The leather treated with such a solution is then placed in a molten mass, the melting point of which is near the boiling point of the solvent which was used in the solution. If benzene is the solvent a melting point of 70 80°-90° C. is selected. Substances suitable for the molten bath are of the kind referred to as being dissolved in the previous example, the most preferable being artificial asphalt, paraffin wax, ceresin and other 75 waxes; with the asphalt oils, varnishes, waxes and the like may be used to fix the required melting point.

The temperature of the molten bath should be above the highest temperature to 80 which the leather will be subjected, for sole leather, for example at least 50° to 60° C. The higher this temperature is, the more solid will be the leather. On introducing the material into the molten mass, there is 85 the tendency for the two liquids to come to equilibrium in accordance with the laws of diffusion. The molten mass therefore wanders through the solvent into the hide and the solvent wanders out. The bath may be 90 kept for the first 24 hours at a temperature of 80° C. so as to let equilibrium be attained by diffusion slowly and without much benzene escaping. The temperature for the next 24 hours may be about 90° to 95°, at 95 which the greater part of the benzene is given off. Care should be taken that during the first hours the temperature of the molten bath does not exceed or only slightly exceeds the boiling point of the solvent, because 100 otherwise the solvent escapes too quickly and so the molten material if this is very viscous, does not sufficiently penetrate the leather. If the mass melts at a very high temperature a suitable pump (rotary pump) 105 may be used for agitating it in the vessel, the vessel itself being evacuated, whereby the desired effect is easily obtained. In this manner the solvent is driven off and sufficient of the molten material penetrates the 110 leather to fill all the pores. This last step may also be effected by placing the hides in a second molten bath free from benzene. In this case it is not necessary to evacuate. The leather is then removed from the bath 115 and the bulk of the contents adhering to it are stripped off and the skin is carefully scraped, the remaining adhering matter being finally washed off with benzene between two brush rollers. It is then finished in any 120 suitable manner and dressed with a thin asphalt varnish. To fill the pores of the leather to the greatest degree, it is advisable to choose a molten material which is soluble in the solvent employed. Otherwise, the solvent will be expelled from the pores in the form of a vapor and the mass will not penetrate into the finest pores to such an extent as when the molten material is soluble in 125 the solvent. However, the use of non-solu- 130

ble materials will produce a good product, especially if the molten mass is quite mobile as is the case when paraffin wax, ceresin or other waxes or artificial asphalt of low melting point is employed. In this case the solvent may be evaporated before the molten mass treatment is carried out or the latter may be carried out without any preceding solution treatment.

10 The hide dehydrated by means of alcohol, whether it is chromed or more or less subjected to any other preliminary tanning or not tanned at all, is characterized by its especially great resistance to high temperatures. But even leathers which have not been dehydrated with alcohol can be subjected to the diffusion process, provided, however, that they have been dehydrated as by being subjected to a high temperature 15 until as much water as possible has been removed from them.

Ordinary chrome leather not dehydrated by means of alcohol, is dried for a short time at 50° C. before being impregnated 20 with the solution, and is then subjected to the above treatment, which however must not last longer than 6 to 8 hours. The leather made in this way from chrome leather differs from other chrome leather by 25 the small amount of filling which it contains.

The tanning with colophony and paraffin wax or ceresin or wax is effected by first 30 impregnating with a benzene solution of 20-50 per cent. strength of colophony which, owing to the low degree of viscosity 35 of the colophony solution attains the maximum of its penetration in a few days; subsequently the hide is immersed in molten 40 paraffin wax, ceresin or wax or in a mixture of these. Accordingly as hard or soft leather is required it is possible to employ varying quantities of one or other of the materials.

45 A special form of the process consists in making objects from the untanned or semi-tanned dried hides and then tanning them or finishing the tanning of them, whereby many advantages are obtained. In the first 50 place the soft or semi-tanned hide is more easily worked than the finished leather, and by subsequently tanning the finished article its resistance to water and damp is increased, especially at the seams. This is of great importance in the shoe uppers and tires for 55 motor road vehicles.

It can be seen that the invention can be carried out in many other modified ways by combining the various parts with each other 60 or with other known methods or known tanning means. This is more especially possible when working with asphalt.

The leather made in accordance with our invention, especially the product of the diffusion method, is characterized by being

water-proof, due both to the complete filling of the hide and to the insolubility of the filling material and by being remarkably stable at high temperatures. Our asphalt leather is capable of withstanding 70 temperatures up to 100° for 48 hours, without damage to its structure and strength. An important feature of the invention which makes for such stability is the complete dehydration of the material by means 75 of a liquid which has an attraction for water. Another valuable property of asphalt leather is that it is serviceable as insulating material for high tension electric currents. A piece 5 m.m. thick is only perforated by a spark produced at a potential of 14,500 volts. This leather is also remarkably resistant to pressure. A load of 2500 kilos square centimeter for five minutes leaves only a scarcely appreciable impression on the loaded part, and this is true whether the leather is dry or wet. Chrome leather filled with an asphaltic base in accordance with our invention has the capacity of holding nails securely, this differing, for instance, from chrome leather filled with paraffin wax.

When, by this new process, colophony and paraffin wax are introduced into chrome leather, owing to the preliminary impregnation with solution, it is possible to introduce in a single operation much more colophony into the hide than by using the molten material alone. According to known methods, the molten material consists of 5 100 to 30 parts of wax or colophony and 95 to 70 parts of paraffin wax or ceresin, while according to the present process a mixture of 70 parts of colophony and 30 parts of paraffin wax can be easily made within the 105 leather. This mixture would not under ordinary circumstances penetrate the dry chrome-leather, at least not at the given temperature of 100° C. and in the course of half an hour to an hour, while according to 110 the new process this is quite possible without any damage to the hide itself.

When in the claims we speak of hides, we mean to include both hides and skins in the 115 untanned state and the same in the tanned state, that is, leather.

When in the claims we speak of resinous matter, we intend to include also the bituminous substances mentioned, which are classed as mineral resins, and such other equivalents 120 as have been hereinbefore enumerated.

We claim:

1. The process of making leather which consists in dehydrating hides by means of a suitable liquid which has an attraction 125 for water and treating the same with a molten mass of resinous matter.

2. The process of making leather which consists in dehydrating chrome leather tanned by any known process, by means of 130

a suitable liquid having an attraction for water and treating the same with a molten mass containing resinous matter.

3. The process of making leather which 5 consists in dehydrating hides by means of a suitable liquid which has an attraction for water and treating the same with a molten mass containing material having an asphaltic base.

10 4. The process of making leather which consists in dehydrating chrome leather tanned by any known process, and treating the same with a molten mass containing material having an asphaltic base.

15 5. The process of making leather which consists in dehydrating hides, treating the same with a solution of resinous matter and subsequently with a molten mass containing resinous matter.

20 6. The process of making leather which consists in dehydrating hides, by means of a suitable liquid having an attraction for water, treating the same with a solution of resinous matter and subsequently with a 25 molten mass containing resinous matter.

7. The process of making leather which consists in dehydrating chrome leather tanned by any known process, treating the same with a solution of resinous matter and 30 subsequently with a molten mass containing resinous matter.

35 8. The process of making leather which consists in dehydrating chrome leather by means of a suitable liquid having an attraction for water, treating the same with a solution of resinous matter and subsequently with a molten mass containing resinous matter.

40 9. The process of making leather which consists in dehydrating hides by means of a suitable liquid having an attraction for water, treating the same with a solution containing material having an asphaltic base and subsequently with a molten mass containing material having an asphaltic base.

45 10. The process of making leather which consists in dehydrating chrome leather by means of a suitable liquid having an attraction for water, treating the same with a 50 solution containing material having an asphaltic base and subsequently with a molten mass containing material having an asphaltic base.

55 11. The process of making leather which consists in dehydrating hides, treating the

same with a solution of resinous matter and subsequently with a molten mass containing material having an asphaltic base.

12. The process of making leather which 60 consists in dehydrating hides by means of a suitable liquid having an attraction for water, treating the same with a solution of resinous matter and subsequently with a molten mass containing material having an asphaltic base.

65 13. The process of making leather which consists in dehydrating chrome leather tanned by any known process, treating the same with a solution of resinous matter and subsequently with a molten mass containing 70 material having an asphaltic base.

14. The process of making leather which 75 consists in dehydrating chrome leather by means of a suitable liquid having an attraction for water, treating the same with a solution of resinous matter and subsequently with a molten mass containing material having an asphaltic base.

15. The process of making leather which 80 consists in dehydrating chrome leather by means of a suitable liquid which has an attraction for water.

16. As a new article of manufacture, the flexible leather, free from fatty impregnated bodies, obtained by treating chrome leather 85 with a suitable liquid having an attraction for water, substantially as described.

17. As a new article of manufacture, the flexible leather, free from fatty impregnated bodies, obtained by treating chrome leather 90 with a suitable liquid having an attraction for water and then treating the thus formed product with resinous matter, substantially as described.

18. As a new article of manufacture, the 95 flexible leather, free from fatty impregnated bodies, obtained by treating chrome leather with a suitable liquid having an attraction for water and then treating the thus formed product with material having an asphaltic 100 base, substantially as described.

In testimony that we claim the foregoing as our invention we have signed our names in presence of two witnesses, this 29th day of November, 1912.

WERNER SPALTEHOLZ.  
KURT HARING.

Witnesses:

FRITZ FISCHER,  
RUDOLPH FRICKE.